

## UNITED STATES PATENT OFFICE.

CARL ADOLPHE KLEIN, OF BRIMSDOWN, AND ROBERT SKIRVING BROWN, OF LONDON, ENGLAND.

## MANUFACTURE OF GLASS, SAND, OR FLINT PAPER, EMERY CLOTH, AND LIKE ABRASIVES.

No Drawing. Application filed October 23, 1925, Serial No. 65,486, and in Great Britain August 26, 1925.

The object of this invention is to provide an improved process for the manufacture of that class of glass, sand or flint paper, emery cloth, and like abrasives, which are water-  
5 proof so that they can be used on damp or wet surfaces without being affected by the moisture.

The invention consists in a series of operations which enable the manufacture to be carried on in a much more practical and commercial manner than by previously known processes.

The invention will be described as applied to the manufacture of waterproof sand paper, and in this case it is preferred to run paper forming the base from a reel, from which it passes (after if desired being printed on the back) into a bath of linseed oil which is kept at a temperature of at least 100° C. A small proportion (say about 0.5 per cent) of paraffin or other suitable wax is added to the linseed oil bath, to increase the waterproofing effect.

From this bath the paper preferably passes between a pair of pressure rollers to remove any surplus of the water-proofing material, and which are also kept heated to 100° C. or over.

It may then be re-wound into reel form, or pass at once direct to a table or series of hot plates or rollers kept at a temperature of 100° C. or over, and while passing over this table or series of hot plates or rollers the adhesive employed to secure the abrasive to the paper is applied in any suitable manner. This adhesive, which consists of a mixture of a drying oil (such as linseed oil or tung oil) with a gum (such as dammar or copal) or synthetic resin, is heated to over 100° C. and applied to the paper while at this temperature.

The following is an example of a suitable composition for this adhesive, viz:

|                        | Parts<br>by weight. |
|------------------------|---------------------|
| 45 Linseed or tung oil | 30                  |
| Dammar or copal gum    | 40                  |

In the sequence of operations the paper thus water-proofed and coated with adhesive passes from the table, hot plates or rollers, and the sand (or other abrasive) is applied in any suitable manner. The paper is then baked at a temperature of over 100° C. Subsequently a second or sizing coating of ad-

hesive is applied, according to common practice, after which the sheet abrasive is rebaked (at a temperature of over 100° C.) and the paper will then be ready for use.

The process above described may be modified by the addition, to the adhesive composition above described, of a small proportion (for instance from 2½ to 5 per cent) of paraffin or other suitable wax. In this case the paper, after passing from the table or hot plates or rollers where the adhesive is applied, is next chilled, after which the abrasive is applied. The paper thus coated passes between hot rollers to press the abrasive down into the warmed adhesive composition, after which it is baked at at least 100° C. as before, but the second or sizing coating of adhesive and the subsequent rebaking will not be necessary.

The various baking operations above referred to may be carried out in an oven or other suitable heating apparatus, and it will be found that the operation will be improved in many cases if a current of heated air is caused to pass therethrough by any suitable means.

It will be obvious that by the use of the process above described the employment of volatile thinners in the waterproofing and adhesive materials is obviated, with the avoidance of the risk of fire and danger to workers from the inhalation of the vapours of such volatile thinners.

What we claim and desire to secure by Letters Patent is:—

1. A process for the manufacture of waterproof sheet abrasive material consisting in waterproofing the base by passing it through a bath of linseed oil containing a small proportion of a suitable wax and kept at a temperature of at least 100° C.; removing any surplus by means of pressure rollers also kept heated to 100° C. or over; applying the adhesive consisting of a mixture of a drying oil with a synthetic resin also at a temperature of over 100° C.; applying the abrasive material to the base thus prepared and baking at a temperature of over 100° C.; and applying a second coating of adhesive and rebaking also at a temperature of over 100° C.

2. A process for the manufacture of waterproof sheet abrasive material consisting in waterproofing the base by passing it through a bath of linseed oil containing a small pro-

portion of a suitable wax and kept at a temperature of at least 100° C.; removing any surplus by means of pressure rollers also kept heated to 100° C. or over; applying the adhesive consisting of a mixture of a drying oil with a synthetic resin in approximately the proportion of 30 parts by weight of oil to 40 parts by weight of resin also at a temperature of over 100° C.; applying the abrasive material to the base thus prepared and baking at a temperature of over 100° C.; and applying a second coating of adhesive and rebaking also at a temperature of over 100° C.

3. A process for the manufacture of water-  
15 proof sheet abrasive material consisting in waterproofing the base by passing it through a bath of linseed oil containing a small proportion of a suitable wax and kept at a temperature of at least 100° C.; removing any  
20 surplus by means of pressure rollers also kept heated to 100° C. or over; applying the adhesive consisting of a mixture of a drying oil with a synthetic resin and a small proportion of paraffin or other suitable wax also at  
25 a temperature of over 100° C.; chilling the

base thus prepared and applying the abrasive; passing the material between hot rollers to press the abrasive into the adhesive composition, and baking at a temperature of 100° C. or over.

30

4. A process for the manufacture of water-  
proof sheet abrasive material consisting in waterproofing the base by passing it through a bath of linseed oil containing a small proportion of a suitable wax and kept at a temperature of at least 100° C.; removing any  
35 surplus by means of pressure rollers also kept heated to 100° C. or over; applying the adhesive consisting of a mixture of a drying oil with a gum and a small proportion of par-  
affin or other suitable wax also at a temperature of over 100° C.; chilling the base thus prepared and applying the abrasive; passing the material between hot rollers to press the abrasive into the adhesive composition, 40 and baking at a temperature of 100° C. or over.

35

In witness whereof we affix our signatures.

CARL ADOLPHIE KLEIN.

ROBERT SKIRVING BROWN.